

May 16, 1961

R. A. BEHN ET AL  
COLOR STABILITY OF SOLVENT TREATED OILS  
AND WAXES DERIVED THEREFROM

2,984,621

Filed Sept. 18, 1958

4 Sheets-Sheet 1

FIG. I



ASTM COLOR  
INVENTORS.  
Robert A. Behn  
Hansford L. Sandlin

*Robert A. Behn*  
*Hansford L. Sandlin*  
Francis T. Johnston  
AGENT.

May 16, 1961

R. A. BEHN ET AL  
COLOR STABILITY OF SOLVENT TREATED OILS  
AND WAXES DERIVED THEREFROM

2,984,621

Filed Sept. 18, 1958

4 Sheets-Sheet 2

FIG. 2



INVENTORS

Robert A. Behn  
Hansford L. Sandlin

by *Francis J. Johnson*

AGENT.

May 16, 1961

R. A. BEHN ET AL  
COLOR STABILITY OF SOLVENT TREATED OILS  
AND WAXES DERIVED THEREFROM

2,984,621

Filed Sept. 18, 1958

4 Sheets-Sheet 3

FIG. 3



INVENTORS.

Robert A. Behn  
Hansford L. Sandlin

by *Francis Johnston*

AGENT.

May 16, 1961

R. A. BEHN ET AL.  
COLOR STABILITY OF SOLVENT TREATED OILS  
AND WAXES DERIVED THEREFROM

2,984,621

Filed Sept. 18, 1958

4 Sheets-Sheet 4



FIG. 4

INVENTORS.

Robert A. Behn  
Tansford L. Sandlin

by *Frances J. Hunter*  
AGENT.

1

2,984,621

## COLOR STABILITY OF SOLVENT TREATED OILS AND WAXES DERIVED THEREFROM

Robert A. Behn and Hansford L. Sandlin, Beaumont, Tex., assignors, by mesne assignments, to Socony Mobil Oil Company, Inc., New York, N.Y., a corporation of New York

Filed Sept. 18, 1958, Ser. No. 761,909

6 Claims. (Cl. 208—370)

The present invention relates to the color stability of solvent treated oils and, more particularly, to the color stability of solvent treated lube oils and the paraffin and microcrystalline waxes derived therefrom. The present invention is particularly related to a method for increasing the filtering capacity of a unit for the percolation of solvent treated lube oils and paraffin and microcrystalline waxes.

In the distillation of crude oil to obtain various products including lubricating oil fractions one of two procedures are generally followed. (1) The crude is distilled to obtain gasoline, kerosene, distillate fuel oil, a paraffin lubricating oil fraction, a microcrystalline lubricating oil fraction, and what is known in the art as a "short resid," or (2) the fractions through distillate fuel oil are vaporized to leave what is known in the art as a "long resid." At this point there is a variation in the further processing which is easily recognized by reference to Figure 4 dependent upon whether the residuum is a "short resid" or a "long resid."

Although solvent treating, dewaxing and percolation of lube oils each is a continuous process the progress of an oil through all three treatments often, and generally, is a discontinuous flow. Thus, while one stock is being solvent treated another stock may be being dewaxed. Consequently, before the second stock can be dewaxed, it is necessary to store the second stock. Frequently, for this and other reasons it is necessary to store stocks for periods up to several days or even two or three weeks or more.

It has been observed that oils darken in storage in an amount sufficient to affect the capacity of the percolation unit. Consequently, the discovery that the color stability of solvent refined oils is affected by the conditions under which the solvent refined oils are stored and the discovery of the conditions under which the color of a solvent refined oil remains substantially constant provides a means for increasing the capacity of a percolation unit as much as 800 percent.

The following discussion in conjunction with the drawings will enable those skilled in the art to understand the present invention. In the following discussion unless specifically noted otherwise, the term "solvent refined lube oil" or "solvent refined lubricating oil" includes all products of the steps in process A and process B subsequent to steps 3a and 3b in process A and all steps subsequent to step 2 in process B and includes the microcrystalline wax of steps 5b in both process A and process B (Figure 4).

In the preparation of finished lube oils it is conventional to treat the lube oil fraction with a solvent. One conventional solvent refining treatment comprises treating the oil with two substantially immiscible solvents such as propane and cresylic acid. This is known as the

2

"Duo-Sol" process. Another solvent treatment comprises treating the lube oil fraction with propane to deasphalt the fraction and treating the deasphalted raffinate with furfural. It is also conventional to dewax the raffinate from any solvent treating process. One of the dewaxing solvents is a mixture of a ketone such as methyl-ethyl ketone and an aromatic solvent such as toluene. The final finishing step is that of percolation through clay such as Attapulgus clay. Often, if not generally, it is necessary to store the treated fraction between successive treatments as between solvent treating and dewaxing and/or between dewaxing and percolating the lube oil fraction. During storage under conditions usually existing the color of the partially treated oil darkens. As is shown in Figure 2 the capacity of a percolation unit is increased if the feed thereto has a lower ASTM color.

Attention is directed to Figure 1 of the drawings. Figure 1 shows graphically the relation between the darkening of the color of a solvent treated oil and the time in storage at a temperature of 180° F. The lube oil fractions the data for which are plotted in Figure 1 were of the types and treated in the manner indicated in Table I.

TABLE I

| Oil No. | Type          | Solvent Refining                     | Dewaxed | Percolated |
|---------|---------------|--------------------------------------|---------|------------|
| 1       | Mid-Continent | "Duo-Sol"                            | Yes     | Yes        |
| 2       | do            | do                                   | No      | No         |
| 3       | do            | do                                   | Yes     | Yes        |
| 4       | Mixed Base    | Propane Deasphalted Furfural Refined | Yes     | No         |
| 5       | Mid-Continent | "Duo-Sol"                            | No      | No         |
| 6       | Coastal       | do                                   | No      | No         |

The various oils were placed in an oven maintained at 180±(2) F. and the color of a sample of each oil determined at various intervals up to 56 days. It will be observed that although there is not a uniform rate at which the color of the oils darkened nevertheless all of the oils darkened to a commercially unacceptable extent. The initial and final colors for each oil are set forth in Table II.

TABLE II

| Oil No. | Initial Dilute ASTM Color | Final Dilute ASTM Color |
|---------|---------------------------|-------------------------|
| 1       | Dark 3                    | Dark 4                  |
| 2       | Lt. 3                     | 3½                      |
| 3       | Lt. 3½                    | Lt. 5                   |
| 4       | Lt. 3                     | Lt. 4½                  |
| 5       | Lt. 3½                    | 4½                      |
| 6       | Lt. 3                     | Lt. 4                   |

Attention is now directed to Figure 2. Figure 2 graphically illustrates the relation between the color of the oil to be percolated and the capacity of the percolation unit. Capacity of the percolation unit is not the barrels of oil which can be treated in a unit time but the amount of oil which can be treated before it is necessary to regenerate the clay. When considering the data presented in Figure 2 it is to be observed that the

colors are rated on two scales, i.e., one scale is for ASTM color when the sample is not diluted and the other of the sample after dilution in accordance with ASTM test procedure. The latter colors are reported as dilute ASTM. Typical of the reduced capacity of a percolation unit between regenerations of the clay is the number of barrels of lube oil fraction having a light 6 ASTM color which can be filtered between regenerations and the number of barrels of lube oil fraction having a light 4½ dilute ASTM color. When both oils are filtered through bauxite at the rate of about 3.8 barrels of oil per hour per 100 cubic feet of clay to obtain a 7 ASTM color the yield of oil from the 6 ASTM color oil is 124 barrels of oil per ton of clay. On the other hand, when the darker oil is filtered the yield is only 14 barrels per ton. Thus, it is apparent that when percolating a lube oil fraction to a 7 ASTM color product the capacity of the unit between regenerations is increased about 800 percent when the color of the fraction to be filtered is not darker than a light 6 ASTM.

The color of the lube oil fraction to be filtered or percolated through bauxite or clay is adversely affected by the temperature to which it is subjected during treatment. Thus, in 10 days at 180° F. the color of a solvent treated lube oil fraction will darken from a light 3 to a 3½ dilute ASTM and in 25 days to 4½ dilute ASTM. On the other hand, at 150° F. the color of the same lube oil fraction will darken from a light 3 dilute ASTM only to a light 3½ dilute ASTM color. Thus, the present invention provides for maintaining the solvent treated lube oil fraction at a temperature not greater than about 150° F. during storage before percolation.

A further improvement in color stability is obtained by control of the gases with which the lube oil fraction is in contact during storage before percolation. Inspection of the curves of Figure 3 makes it manifest that the color of a lube oil fraction darkens much more rapidly when stored in contact with air than when stored in contact with a non-oxidizing gas such as nitrogen, natural gas or flue gas substantially devoid of oxygen. In fact, curve "A" in Figure 3 shows that if a lube oil fraction is stored even at 180° F. under a blanket of non-oxidizing gas the color remains substantially constant for at least 32 days.

It has also been discovered that the color of micro-crystalline wax admixed with oil, generally known to the art as petrolatum, is improved and stabilized when it

is necessary to store the petrolatum by storing the petrolatum under a blanket of non-oxidizing gas such as nitrogen, natural gas or flue gas substantially devoid of oxygen even though the petrolatum is stored at 180° F.

Solvent refined oil and petrolatum having the physical properties set forth in Table III were stored under blankets of gases having the compositions set forth in Table IV.

TABLE III  
Physical properties of stock 330 raffinate and petrolatum

|                              | Sample | Stock 330 Raffinate | Petrolatum |
|------------------------------|--------|---------------------|------------|
| 15                           |        |                     |            |
| Gravity, °API.....           |        | 27.7                | 34.0       |
| Color, NPA.....              |        | D.6                 | D.7        |
| Viscosity, SUS @ 210° F..... |        | 136                 | 109        |
| C.C.R., Wt. Percent.....     |        | 0.45                | 0.30       |

TABLE IV  
Analyses of gases used for blanketing

|                                         | Composition | Vol. Percent | Flue Gas <sup>1</sup> | Flue Gas <sup>2</sup> | Natural Gas <sup>3</sup> |
|-----------------------------------------|-------------|--------------|-----------------------|-----------------------|--------------------------|
| CO <sub>2</sub> .....                   | 9.2         | 11.6         | 11.0                  | 0.9                   |                          |
| O <sub>2</sub> .....                    | 6.7         | 0            | 0.8                   | -----                 |                          |
| CO.....                                 | 0           | 0            | 0                     | -----                 |                          |
| 30 N <sub>2</sub> and Other Inerts..... | 76          | 87.2         | 88.2                  | -----                 |                          |
| H <sub>2</sub> .....                    |             |              |                       |                       | 0.4                      |
| H <sub>2</sub> S.....                   |             |              |                       |                       | 0.1                      |
| Cl <sub>1</sub> .....                   |             |              |                       |                       | 98.6                     |

<sup>1</sup> Oxygen free flue gas.

<sup>2</sup> Flue gas with 0.8% Oxygen.

<sup>3</sup> Purchased natural gas.

It will be observed that flue gas as usually produced contains an appreciable amount of oxygen. A typical analysis of flue gas is given here below.

|                                       | FLUE GAS | Volume percent |
|---------------------------------------|----------|----------------|
| CO <sub>2</sub> .....                 |          | 10.1           |
| O <sub>2</sub> .....                  |          | 3.5            |
| 45 CO .....                           |          | 0              |
| N <sub>2</sub> and other inerts ..... |          | 86.4           |

The color of the solvent refined oil degraded with time when blanketed by the gases the compositions of which are given in Table IV as shown in Table V.

TABLE V

Color stability of stock solvent refined lube oil blanketed with air, flue gases and natural gas

[Stored at 180° F. in sealed 4-oz. bottles]

| Blanketed Material | Air    |            | Flue gas, 0.8 O <sub>2</sub> |            | Flue Gas, no O <sub>2</sub> |            | Natural gas |            |
|--------------------|--------|------------|------------------------------|------------|-----------------------------|------------|-------------|------------|
|                    | NPA    | Dilute NPA | NPA                          | Dilute NPA | NPA                         | Dilute NPA | NPA         | Dilute NPA |
| Days in Storage:   |        |            |                              |            |                             |            |             |            |
| Start.....         | D.6    | 3½         | D.6                          | 3½         | D.6                         | 3½         | D.6         | 3½         |
| 7.....             | 4      | D.6        | 4                            | D.6        | D.7                         | 3½         | 8           | 4          |
| 14.....            | 4      | D.6        | 4                            | D.6        | D.7                         | 3½         | D.8         | 4          |
| 21.....            | 4½     | D.7        | 4½                           | D.7        | D.7                         | D.3½       | D.8         | 4          |
| 28.....            | 4½     | D.7        | 4½                           | D.7        | D.7                         | D.3½       | D.8         | 4          |
| 35.....            | 4½     | D.7        | 4½                           | D.7        | D.7                         | D.3½       | D.8         | 4          |
| 42.....            | 4½     | D.7        | 4½                           | D.7        | D.7                         | D.3½       | D.8         | 4          |
| 49.....            | 4½     | D.7        | 4½                           | D.7        | D.7                         | D.3½       | D.8         | 4          |
| 56.....            | Black. | D.8        | Black.                       | D.8        | D.7                         | D.3½       | D.8         | 4          |
| 63.....            | Black. | D.8        | Black.                       | D.8        | 4                           | D.7        | 4           | D.8        |
| 70.....            | Black. | TR         | Black.                       | D.8        | 4                           | D.7        | 4           | D.8        |

TR=Transparent red (darker than 8).

The color of the petrolatum obtained from the solvent refined oil degraded with time when blanketed with the gases of Table IV as set forth in Table VI.

TABLE VI

*Color stability of petrolatum from solvent refined lube oil (Table IV) blanketed with air and flue gas*  
[Stored at 180° F. in sealed 4-oz. bottles]

| Blanketing Material | Air  |            | Containing no O <sub>2</sub> Flue Gas |            |
|---------------------|------|------------|---------------------------------------|------------|
|                     | NPA  | Dilute NPA | NPA                                   | Dilute NPA |
| Days in Storage:    |      |            |                                       |            |
| Start               |      |            |                                       |            |
| 7                   | D. 7 | 3½-        | D. 7                                  | 3½-        |
| 14                  | D. 8 | 4-         | D. 7                                  | 3½-        |
| 21                  | D. 8 | 4-         | D. 7                                  | 3½-        |
| 28                  | D. 8 | D. 4       | D. 7                                  | 3½-        |
| 35                  | TR   | 4½-        | D. 7                                  | 3½-        |
| 42                  | TR   | 5-         | D. 7                                  | D. 3½-     |
| 49                  | TR   | 5-         | D. 7                                  | D. 3½-     |
| 56                  | TR   | 5-         | 8-                                    | 4-         |
| 63                  | TR   | 5-         | 8-                                    | 4-         |
| 70                  | TR   | 5+         | 8                                     | 4-         |

The results set forth in Tables V and VI are summarized in Table VII.

TABLE VII

|                                                                 | Dilute NPA Color    |            |
|-----------------------------------------------------------------|---------------------|------------|
|                                                                 | Stock 830 Raffinate | Petrolatum |
| Sample Before Storage                                           | 3½-                 | 3½-        |
| Sample After Storage for 70 Days at 180° F.,<br>Blanketed With: |                     |            |
| Air                                                             | TR                  | Dk. 5      |
| Flue Gas—No O <sub>2</sub>                                      | 4-                  | 4-         |
| Flue Gas—0.8% O <sub>2</sub>                                    | 4-                  | 4-         |
| Natural Gas                                                     | 4-                  | 4-         |

The summary given in Table VII clearly establishes that natural gas, flue gas containing no oxygen, and flue gas containing not more than 1 percent by volume of oxygen are equally effective in reducing the color degradation of both solvent refined oil and the petrolatum obtained therefrom.

The effect of small differences in color upon the yield of microcrystalline wax of required color is outstanding as even cursory examination of the data presented in Table X will establish.

The microcrystalline waxes obtained from the afore-described petrolatum had the physical properties listed in Table VIII.

TABLE VIII

*Physical properties of microcrystalline waxes*

|                            |      |      |      |
|----------------------------|------|------|------|
| Gravity, °API              | 33.2 | 34.3 | 34.3 |
| Color, NPA Dilute          | 5-   | 4½-  | 3½-  |
| Viscosity, SUS @ 210° F.   | 120  | 96   | 96   |
| Water Content, Wt. Percent | Nil  | Nil  | Nil  |

The bauxite through which the microcrystalline waxes were percolated had the physical properties given in Table IX.

TABLE IX

*Physical properties of bauxite:*

|                                |      |
|--------------------------------|------|
| Density, lbs./ft. <sup>3</sup> | 66.3 |
| Volatile matter, wt. percent   | 0.63 |

## SCREEN ANALYSIS

| Screen size: | Wt. percent retained |
|--------------|----------------------|
| 16           | 0.1                  |
| 20           | 0.1                  |
| 30           | 13.9                 |
| 40           | 18.9                 |
| 50           | 42.9                 |
| 60           | 10.0                 |
| 65           | 6.1                  |
| 100          | 5.8                  |
| 100+         | 2.2                  |

The yields of percolated wax in pounds of wax filtered per ton of bauxite to produce microcrystalline having a color not darker than NPA 5 are given in Table X.

TABLE X

*Percolation of different color microcrystalline waxes*

| 5—Dilute NPA Charge | 4½—Dilute NPA Charge | 3½—Dilute NPA Charge | Filter Yield, Bbls./Ton |                     | Composite NPA Color     |                     |
|---------------------|----------------------|----------------------|-------------------------|---------------------|-------------------------|---------------------|
|                     |                      |                      | Filter Yield, Bbls./Ton | Composite NPA Color | Filter Yield, Bbls./Ton | Composite NPA Color |
| 2.23                | 1½                   | 1.85                 | 1½+                     | 2.23                | 1½                      |                     |
| 4.46                | 2-                   | 3.15                 | 2-                      | 4.46                | 2-                      |                     |
| 6.69                | 3+                   | 4.51                 | 2½+                     | 6.69                | 3-                      |                     |
| 8.92                | 4-                   | 5.80                 | 3½                      | 8.92                | 3+                      |                     |
| 11.16               | 4½                   | 7.17                 | 4-                      | 11.16               | 3½+                     |                     |
| 13.39               | 5-                   | 8.46                 | 4-                      | 13.39               | 3½+                     |                     |
| 13.95               | 5                    | 9.76                 | 4+                      | 15.62               | 4                       |                     |
|                     |                      | 11.12                | 4½+                     | 17.85               | 4+                      |                     |
|                     |                      | 12.42                | 4½+                     | 20.08               | 4½-                     |                     |
|                     |                      | 13.74                | 4½+                     | 22.32               | 4½                      |                     |
|                     |                      | 15.13                | 5-                      | 24.55               | 4½+                     |                     |
|                     |                      | 16.52                | 5-                      | 26.78               | 4½+                     |                     |
|                     |                      | 17.90                | 5                       | 29.01               | 4½+                     |                     |
|                     |                      |                      |                         | 31.24               | 5-                      |                     |
|                     |                      |                      |                         | 33.48               | 5-                      |                     |
|                     |                      |                      |                         | 35.71               | 5-                      |                     |
|                     |                      |                      |                         | 37.94               | 5-                      |                     |
|                     |                      |                      |                         | 40.17               | 5-                      |                     |
|                     |                      |                      |                         | 42.40               | 5-                      |                     |
|                     |                      |                      |                         | 44.64               | 5-                      |                     |
|                     |                      |                      |                         | 46.87               | 5-                      |                     |
|                     |                      |                      |                         | 49.10               | 5                       |                     |

The data presented in Table X are summarized in Table XI.

TABLE XI

| Color of Charge Stock NPA Dilute | Yield of Intermediate Grade Wax of 5 NPA Composite Color, Bbls./Ton of Bauxite |
|----------------------------------|--------------------------------------------------------------------------------|
| 5-                               | 14                                                                             |
| 4½-                              | 18                                                                             |
| 3½-                              | 49                                                                             |

Accordingly, the present invention provides a means for increasing the capacity between regenerations of a percolation unit for filtering solvent refined lube oil fractions and waxes obtained therefrom by (1) maintaining the lube oil fraction and the waxes obtained therefrom between treatments or during storage before percolation and after percolation at a temperature not greater than about 150° F.; (2) by blanketing the lube oil fraction between treating steps or during storage before percolation with a non-oxidizing gas such as natural gas, flue gas containing not more than about 1 percent by volume of oxygen, nitrogen, etc. while maintaining the temperature below about 200° F.; and (3) by maintaining the temperature of a lube oil fraction not higher than 150° F. and blanketing the lube oil fraction with a non-oxidizing gas such as natural gas, flue gas containing not more than about 1 percent by volume of oxygen, nitrogen, etc. As used in the claims, intermediate storage before percolation designates storage between

successive treatments as between solvent refining and dewaxing or between dewaxing and percolation.

This application is a continuation-in-part of copending application Serial No. 677,901, filed August 13, 1957.

We claim:

1. In the refining of a lubricating oil fraction of a mineral oil comprising the steps in succession of (a) solvent extraction, (b) dewaxing, and (c) percolation through clay, wherein a partially refined portion of said fraction is stored following one of said treatments but before percolation through clay, the method of stabilizing the color of said partially refined portion during storage which comprises maintaining said stored portion in a fluid state at a temperature below about 200° F. while under a blanket of non-oxidizing gas.

2. The process according to claim 1 in which the stored portion is a dewaxed raffinate.

3. The method according to claim 1 in which the non-oxidizing gas is flue gas substantially devoid of oxygen.

4. The method according to claim 1 in which the stored portion is a solvent extracted lube oil.

5. The method according to claim 1 in which the stored portion is petrolatum.

6. The method according to claim 1 in which the stored portion is microcrystalline wax.

10

15

**References Cited in the file of this patent**

**UNITED STATES PATENTS**

|           |                 |               |
|-----------|-----------------|---------------|
| 2,045,160 | Moorman et al.  | June 23, 1936 |
| 2,106,071 | Stanton         | Jan. 18, 1938 |
| 2,321,459 | Chenault et al. | June 8, 1943  |
| 2,728,716 | Watson et al.   | Dec. 27, 1955 |
| 2,862,876 | Winberg         | Dec. 2, 1958  |